# EUROPEAN PATENT SPECIFICATION

(11) **EP 1 767 349 B1**
(45) Date of publication and mention of the grant of the patent: **23.07.2008**
(21) Application number: 05108920.9
(22) Date of filing: 27.09.2005
(51) Int. Cl.: B41C 1/10

(54) **Method for making a lithographic printing plate**
Verfahren zur Herstellung einer lithographischen Druckplatte
Procédé de production d'une plaque d'impression lithographique

(43) Date of publication of application: 28.03.2007
(73) Proprietor: Agfa Graphics N.V., 2640 Mortsel (BE)
(72) Inventor: Verschueren, Eric, 2640, Mortsel (BE)
(74) Representative: Goedeweeck, Rudi

(56) References cited:
- EP-A- 0 770 494
- EP-A- 0 839 648
- EP-A- 1 243 413
- EP-A- 1 506 854

## Description

### FIELD OF THE INVENTION

The present invention relates to a method for making a wet lithographic printing plate by exposing a heat-sensitive, negative working lithographic printing plate precursor to infrared light, developing the exposed precursor and then subjecting the plate to a mild baking step.

### BACKGROUND OF THE INVENTION

Lithographic printing presses use a so-called printing master such as a printing plate which is mounted on a cylinder of the printing press. The master carries a lithographic image on its surface and a print is obtained by applying ink to said image and then transferring the ink from the master onto a receiver material, which is typically paper. In conventional, so-called "wet" lithographic printing, ink as well as an aqueous fountain solution (also called dampening liquid) are supplied to the lithographic image which consists of oleophilic (or hydrophobic, i.e. ink-accepting, water-repelling) areas as well as hydrophilic (or oleophobic, i.e. water-accepting, ink-repelling) areas. In so-called driographic printing, the lithographic image consists of ink-accepting and ink-abhesive (ink-repelling) areas and during driographic printing, only ink is supplied to the master.

Printing masters are generally obtained by the image-wise exposure and processing of an imaging material called plate precursor. In addition to the well-known photosensitive, so-called pre-sensitized plates, which are suitable for UV contact exposure through a film mask, also heat-sensitive printing plate precursors have become very popular in the late 1990s. Such thermal materials offer the advantage of daylight stability and are especially used in the so-called computer-to-plate method wherein the plate precursor is directly exposed, i.e. without the use of a film mask. The material is exposed to heat or to infrared light and the generated heat triggers a (physico-)chemical process, such as ablation, polymerization, insolubilization by crosslinking of a polymer, heat-induced solubilization, or by particle coagulation of a thermoplastic polymer latex.

Although some of these thermal processes enable plate making without wet processing, the most popular thermal plates form an image by a heat-induced solubility difference in an alkaline developer between exposed and non-exposed areas of the coating. The coating typically comprises an oleophilic binder, e.g. a phenolic resin, of which the rate of dissolution in the developer is either reduced (negative working) or increased (positive working) by the image-wise exposure. During processing, the solubility differential leads to the removal of the non-image (non-printing) areas of the coating, thereby revealing the hydrophilic support, while the image (printing) areas of the coating remain on the support. Negative working embodiments of such thermal materials often require a preheat step between exposure and development as described in e.g. EP-A 625,728.

Negative working plate precursors which do not require a preheat step may contain an image-recording layer that works by heat-induced particle coalescence of a thermoplastic polymer latex, as described in e.g. EP-A's 770 494, 770 495, 770 496 and 770 497. These patents disclose a method for making a lithographic printing plate comprising the steps of (1) image-wise exposing a plate precursor having a heat-sensitive image-recording layer to infrared light, wherein said image-recording layer comprises hydrophobic thermoplastic polymer particles, sometimes also referred to as latex particles, which are dispersed in a hydrophilic binder, and (2) developing the image-wise exposed element by applying water or by mounting the plate on the plate cylinder of a press and then supplying fountain and/or ink. During the development step, the unexposed areas of the image-recording layer are removed from the support, whereas the latex particles in the exposed areas have coalesced to form a hydrophobic phase which is not removed in the development step. In EP-A 1 342 568 a similar plate precursor is developed with a gum solution and in unpublished EP-A's no. 04103245, 04103247 and 04103248, all filed on 8 July 2004, development is achieved by means of an alkaline solution.

It is known in the art that lithographic plates, obtained after exposure, development and optional gumming, can be heat-treated in a so-called post-baking step in order to increase the run length of the plate on the press. A typical post-baking is carried out by heating the plate in an oven at a high temperature, e.g. of about 250°C.
EP-A 1 506 854 describes a method for post-baking various plates, including plates that work by heat-induced latex coalescence, in a short time of 1 minute or less by means of an infrared radiation source.

A problem associated with plate precursors that work according to the mechanism of heat-induced latex coalescence is that it is difficult to obtain both a high sensitivity enabling exposure at a low energy density, and a good clean-out of the unexposed areas during development. The energy density that is required to obtain a sufficient degree of latex coalescence and of adherence of the exposed areas to the support is often higher than 250 mJ/cm². As a result, in platesetters that are equipped with low power exposure devices such as semiconductor infrared laser diodes, such materials require long exposure times.

A higher sensitivity can be obtained e.g. by providing an image-recording layer that has a better resistance towards the developer in the unexposed state, so that a low energy density suffices to render the image-recording layer completely resistant to the developer. However, such an image-recording layer is difficult to remove during development and results in toning (ink acceptance in the non-image areas). This toning especially occurs when the plate is baked after development. Another way to provide a higher sensitivity can be achieved by using latex particles that are only weakly stabilized so that they coalesce readily i.e. upon exposure at a low energy density. However, such latex particles tend to remain on the support also in the unexposed state and again, an insufficient clean-out (removal of the coating during development) is obtained, resulting in toning.

On the other hand, well-stabilized latex particles are easily removed from the support and show no clean-out problems but they require more energy to coalesce and thus a low sensitivity plate is obtained.

### SUMMARY OF THE INVENTION

It is an object of the present invention to provide a negative-working lithographic printing plate precursor that works by heat-induced coalescence of thermoplastic polymer particles, which enables both (i) a short exposure time on low power plate setters, and (ii) a good clean-out of the unexposed areas during development resulting in plates which show no toning.

This object is realized by the method defined in claim 1, having the specific features that the precursor is exposed at an energy density of 190 mJ/cm² or less, and that the precursor is then subjected to a mild post-baking step, more particularly to a post-baking step between 5 seconds and 2 minutes.

It was suprisingly found that an energy density of 190 mJ/cm² or less, which is typically too low for providing a good adherence of the exposed areas to the support, nevertheless is sufficient to render the exposed areas resistant to the development step. Without prejudice to the scope of our claims, it seems that the mild post-baking step compensates for the underexposure, as explained hereafter. The energy density of 190 mJ/cm² seems to be sufficient to provide enough differentiation between exposed and unexposed areas to obtain a high-quality lithographic image after development, i.e. a complete clean-out of the unexposed areas without substantially affecting the exposed areas. However, the mechanical and chemical resistance of the (underexposed) lithographic image is insufficient to provide an acceptable run length of the plate during printing According to the present invention, that problem is solved by the mild post-baking step; i.e. a post baking step between 5 seconds and 2 minutes.

As an additional benefit, the plate-making time is reduced by the combination of both a short exposure time and a short post-baking step. Furthermore, the short post-baking step also reduces the risk of distortion of the support which is often observed after a conventional post-baking step.

Traditionally, baking is carried out by keeping the developed plate in an oven. The advantages of the method of our invention enable to provide a preferred embodiment wherein all steps are carried out in an integrated plate-making apparatus. The integrated plate-making apparatus comprises a plate-setter, a processing unit and a baking unit. According to said preferred embodiment, the plate precursor which has been exposed in the plate-setter is mechanically conveyed to the processing unit which is coupled to the plate-setter. After developing the exposed plate in the processing unit, the developed plate is then mechanically conveyed from the processing unit to a baking unit. The short baking step according to the present invention allows the use of a small baking unit so that the developed plate is directly conveyed from the processing unit into said baking unit. The plate then travels through the baking unit and leaves said unit within a time period of two minutes or less.

In a preferred embodiment, the baking unit comprises a cooling zone so that the plate temperature is reduced before the plate leaves the baking unit. The baking unit is preferably equipped with an exhaust to remove volatile compounds that are released by the plate material. The exhaust preferably comprises an easily exchangeable filter.

Other preferred embodiments of the method of the present invention are further defined in the dependent claims.

### BRIEF DESCRIPTION OF THE DRAWINGS

Fig. 1 shows a schematic diagram of a gumming unit.
Fig. 2 shows a schematic diagram of an integrated plate-making apparatus.
Fig. 3 shows the rendering of a 10% screen of 200lpi (lines per inch lpi or about 80 lines/cm) on a printed copy produced with the comparative printing plates 1 and 2 and invention printing plate 3 (see Examples: Print results).

### DETAILED DESCRIPTION OF THE INVENTION

The support of the lithographic printing plate precursor used in the method of the present invention has a hydrophilic surface or is provided with a hydrophilic layer. The support may be a sheet-like material such as a plate or it may be a cylindrical element such as a sleeve which can be slid around a print cylinder of a printing press. Preferably, the support is a metal support such as aluminum or stainless steel. The support can also be a laminate comprising an aluminum foil and a plastic layer, e.g. polyester film.

A particularly preferred lithographic support is an electrochemically grained and anodized aluminum support. The aluminum is preferably grained by electrochemical graining, and anodized by means of anodizing techniques employing phosphoric acid or a sulphuric acid/phosphoric acid mixture. Methods of both graining and anodization of aluminum are very well known in the art. By graining (or roughening) the aluminium support, both the adhesion of the printing image and the wetting characteristics of the non-image areas are improved. By varying the type and/or concentration of the electrolyte and the applied voltage in the graining step, different type of grains can be obtained. By anodising the aluminium support, its abrasion resistance and hydrophilic nature are improved. The microstructure as well as the thickness of the Al₂O₃ layer are determined by the anodising step, the anodic weight (g/m² A1203 formed on the aluminium surface) may vary between 1 and 8 g/m².

The grained and anodized aluminum support may be post-treated to improve the hydrophilic properties of its surface. For example, the aluminum oxide surface may be silicated by treating its surface with a sodium silicate solution at elevated temperature, e.g. 95°C. Alternatively, a phosphate treatment may be applied which involves treating the aluminum oxide surface with a phosphate solution that may further contain an inorganic fluoride. Further, the aluminum oxide surface may be rinsed with an organic acid and/or salt thereof, e.g. carboxylic acids, hydrocarboxylic acids, sulphonic acids or phosphonic acids, or their salts, e.g. succinates, phosphates, phosphonates, sulphates, and sulphonates. A citric acid or citrate solution is preferred. This treatment may be carried out at room temperature or may be carried out at a slightly elevated temperature of about 30°C to 50°C. A further interesting treatment involves rinsing the aluminum oxide surface with a bicarbonate solution. Still further, the aluminum oxide surface may be treated with polyvinylphosphonic acid, polyvinylmethylphosphonic acid, phosphoric acid esters of polyvinyl alcohol, polyvinylsulfonic acid, polyvinylbenzenesulfonic acid, sulfuric acid esters of polyvinyl alcohol, and acetals of polyvinyl alcohols formed by reaction with a sulfonated aliphatic aldehyde. It is further evident that one or more of these post treatments may be carried out alone or in combination. More detailed descriptions of these treatments are given in GB 1084070, DE 4423140, DE 4417907, EP 659909, EP 537633, DE 4001466, EP A 292801, EP A 291760 and US 4458005.

According to another embodiment, the support can also be a flexible support, which is provided with a hydrophilic layer, hereinafter called 'base layer'. The flexible support is e.g. paper, plastic film, thin aluminum or a laminate thereof. Preferred examples of plastic film are polyethylene terephthalate film, polyethylene naphthalate film, cellulose acetate film, polystyrene film, polycarbonate film, etc. The plastic film support may be opaque or transparent.

The base layer is preferably a cross-linked hydrophilic layer obtained from a hydrophilic binder cross-linked with a hardening agent such as formaldehyde, glyoxal, polyisocyanate or a hydrolyzed tetra-alkylorthosilicate. The latter is particularly preferred. The thickness of the hydrophilic base layer may vary in the range of 0.2 to 25 µm and is preferably 1 to 10 µm. The hydrophilic binder for use in the base layer is e.g. a hydrophilic (co)polymer such as homopolymers and copolymers of vinyl alcohol, acrylamide, methylol acrylamide, methylol methacrylamide, acrylate acid, methacrylate acid, hydroxyethyl acrylate, hydroxyethyl methacrylate or maleic anhydride/vinylmethylether copolymers. The hydrophilicity of the (co)polymer or (co)polymer mixture used is preferably the same as or higher than the hydrophilicity of polyvinyl acetate hydrolyzed to at least an extent of 60% by weight, preferably 80% by weight. The amount of hardening agent, in particular tetra-alkyl orthosilicate, is preferably at least 0.2 parts per part by weight of hydrophilic binder, more preferably between 0.5 and 5 parts by weight, most preferably between 1 parts and 3 parts by weight.

According to another embodiment the base layer may also comprise Al₂O₃ and an optional binder. Deposition methods for the Al₂O₃ onto the flexible support may be (i) physical vapor deposition including reactive sputtering, RF-sputtering, pulsed laser PVD and evaporation of aluminium, (ii) chemical vapor deposition under both vacuum and non-vacuum condition, (iii) chemical solution deposition including spray coating, dipcoating, spincoating, chemical bath deposition, selective ion layer adsorption and reaction, liquid phase deposition and electroless deposition. The Al₂O₃ powder can be prepared using different techniques including flame pyrolisis, ball milling, precipitation, hydrothermal synthesis, aerosol synthesis, emulsion synthesis, sol-gel synthesis (solvent based), solution-gel synthesis (water based) and gas phase synthesis. The particle size of the Al₂O₃ powders can vary between 2 nm and 30 µm; more preferably between 100 nm and 2 µm.

The hydrophilic base layer may also contain substances that increase the mechanical strength and the porosity of the layer. For this purpose colloidal silica may be used. The colloidal silica employed may be in the form of any commercially available water dispersion of colloidal silica for example having a particle size up to 40 nm, e.g. 20 nm. In addition inert particles of larger size than the colloidal silica may be added e.g. silica prepared according to Stöber as described in J. Colloid and Interface Sci., Vol. 26, 1968, pages 62 to 69 or alumina particles or particles having an average diameter of at least 100 nm which are particles of titanium dioxide or other heavy metal oxides.

Particular examples of suitable hydrophilic base layers for use in accordance with the present invention are disclosed in EP 601240, GB 1419512, FR 2300354, US 3971660, and US 4284705.

The coating on the support comprises hydrophobic thermoplastic particles. The coating may comprise one or more layer(s) and the layer comprising the hydrophobic thermoplastic particles is referred to herein as 'image-recording layer'. The weight average molecular weight of the thermoplastic polymer particles may range from 5,000 to 1,000,000 g/mol. The hydrophobic particles preferably have a number average particle diameter below 200 nm, more preferably between 10 and 100 nm. In a specific embodiment, the average particle size is comprised between 40 nm and 70 nm, more preferably between 45 nm and 65 nm. The particle size is defined herein as the particle diameter, measured by Photon Correlation Spectrometry, also known as Quasi-Elastic or Dynamic Light-Scattering. This technique produces values of the particle size that match well with the particle size measured with transmission electronic microscopy (TEM) as disclosed by Stanley D. Duke et al. in Calibration of Spherical Particles by Light Scattering, in Technical Note-002B, May 15, 2000 (revised 1/3/2000 from a paper published in Particulate Science and Technology 7, p. 223-228 (1989). An optimal ratio between the pore diameter of the hydrophilic surface of the aluminum support (if present) and the average particle size of the hydrophobic thermoplastic particles may enhance the press run length of the plate and may improve the toning behaviour of the prints. The ratio of the average pore diameter of the hydrophilic surface of the aluminum support to the average particle size of the polymer particles preferably ranges from 0.05:1 to 0.8:1, more preferably from 0.10:1 to 0.35:1.

The amount of hydrophobic thermoplastic polymer particles contained in the image-recording layer is preferably between 20 and 90 percent by weight (wt.%), relative to the weight of all the components in the image-recording layer. In a preferred embodiment, the amount of hydrophobic thermoplastic polymer particles present in the image-recording layer is at least 70 wt.% and more preferably at least 75 wt.%. An amount between 75 and 85 wt.% produces excellent results.

Suitable examples of polymers present in the hydrophobic thermoplastic polymer particles are polyethylene, poly(vinyl)chloride, polymethyl(meth)acrylate , polyethyl (meth)acrylate, poyvinylidene chloride, poly(meth)acrylonitrile, polyvinylcarbazole, polystyrene or copolymers thereof. According to a preferred embodiment, the thermoplastic polymer particles comprise polystyrene or derivatives thereof. Mixtures comprising polystyrene or derivatives thereof and copolymers of styrene or derivatives thereof are most preferred.

In order to obtain sufficient resistivity towards organic chemicals such as hydrocarbons used in plate cleaners, the hydrophobic thermoplastic polymer particles preferably comprise nitrogen containing monomeric units or units which correspond to monomers that are characterized by a solubility parameter larger than 20, such as (meth)acrylonitrile or monomeric units comprising sulfonamide and/or phthalimide pendant groups. Other suitable examples of such units are disclosed in EP 1,219,416. The average amount of said units is at least 5 wt.%, more preferably at least 30 wt.% of the polymer particle.

A preferred embodiment of the hydrophobic thermoplastic polymer is a copolymer comprising polystyrene and poly(meth)acrylonitrile or derivatives thereof. The latter copolymers may comprise at least 50% by weight of polystyrene, and more preferably at least 65% by weight of polystyrene. According to the most preferred embodiment, the thermoplastic polymer particles consist essentially of styrene and acrylonitrile units in a weight ratio between 1:1 and 5:1 (styrene:acrylonitrile), e.g. in a 2:1 ratio.

The hydrophobic thermoplastic polymer particles present in the image-recording layer can be applied onto the lithographic base in the form of a dispersion in an aqueous coating liquid and may be prepared by the methods disclosed in US 3,476,937 or EP 1,217,010. Another method especially suitable for preparing an aqueous dispersion of the thermoplastic polymer particles comprises:
- dissolving the hydrophobic thermoplastic polymer in an organic water immiscible solvent,
- dispersing the thus obtained solution in water or in an aqueous medium and
- removing the organic solvent by evaporation.

The image-recording layer further comprises a hydrophilic binder. Examples of suitable hydrophilic binders are homopolymers and copolymers of vinyl alcohol, acrylamide, methylol acrylamide, methylol methacrylamide, acrylic acid, methacrylic acid, hydroxyethyl acrylate, hydroxyethyl methacrylate and maleic anhydride/vinylmethylether copolymers.

The coating also contains a compound which absorbs infrared light and converts the absorbed energy into heat. The amount of infrared absorbing agent in the coating is preferably between 0.25 and 25.0 % by weight, more preferably between 0.5 and 20.0 % by weight. The infrared absorbing compound can be present in the image-recording layer and/or an optional other layer. In the embodiment wherein the infrared absorbing agent is present in the image-recording layer of the coating, its concentration is preferably at least 6 % by weight, more preferably at least 8 % by weight, relative to the weight of all the components in the image-recording layer. Preferred IR absorbing compounds are dyes such as cyanine, merocyanine, indoaniline, oxonol, pyrilium and squarilium dyes or pigments such as carbon black. Examples of suitable IR absorbers are described in e.g. EP-As 823327, 978376, 1029667, 1053868, 1093934; WO 97/39894 and 00/29214. A preferred compound is the following cyanine dye IR-1 or a suitable salt thereof:

To protect the surface of the coating, in particular from mechanical damage, a protective layer may also optionally be applied. The protective layer generally comprises at least one water-soluble polymeric binder, such as polyvinyl alcohol, polyvinylpyrrolidone, partially hydrolyzed polyvinyl acetates, gelatin, carbohydrates or hydroxyethylcellulose, and can be produced in any known manner such as from an aqueous solution or dispersion which may, if required, contain small amounts of organic solvents, e.g. less than 5% by weight, based on the total weight of the coating solvents for the protective layer. The thickness of the protective layer can suitably be any amount, advantageously up to 5.0 µm, preferably from 0.05 to 3.0 µm, particularly preferably from 0.10 to 1.0 µm.

Besides the additional layers already discussed above - i.e. an optional light-absorbing layer comprising one or more compounds that are capable of converting infrared light into heat and/or a protective layer such as e.g. a covering layer which is removed during processing - the coating may further comprise other additional layer(s) such as for example an adhesion-improving layer between the image-recording layer and the support.

Optionally, the coating may further contain additional ingredients. These ingredients may be present in the image-recording layer or in on optional other layer. For example, additional binders, polymer particles such as matting agents and spacers, surfactants such as perfluoro surfactants, silicon or titanium dioxide particles, development inhibitors, development accelerators or colorants are well-known components of lithographic coatings. Especially addition of colorants such as dyes or pigments which provide a visible color to the coating and remain in the exposed areas of the coating after the processing step, are advantageous. Thus, the image-areas which are not removed during the processing step form a visible image on the printing plate and examination of the developed printing plate already at this stage becomes feasible. Typical examples of such contrast dyes are phthalocyanines or the amino-substituted tri- or diarylmethane dyes, e.g. crystal violet, methyl violet, victoria pure blue, flexoblau 630, basonylblau 640, auramine and malachite green. Also the dyes which are discussed in depth in the detailed description of EP-A 400,706 are suitable contrast dyes. Dyes which, combined with specific additives, only slightly color the coating but which become intensively colored after exposure, are also of interest.

The printing plate precursor of the present invention is image-wise exposed by infrared light, preferably near infrared light. The infrared light is preferably converted into heat by an IR light absorbing compound as discussed above. The heat-sensitive lithographic printing plate precursor of the present invention is preferably not sensitive to visible light. Most preferably, the coating is not sensitive to ambient daylight, i.e. visible (400-750 nm) and near UV light (300-400 nm) at an intensity and exposure time corresponding to normal working conditions so that the material can be handled without the need for a safe light environment.

The printing plate precursors of the present invention can be exposed to infrared light by means of e.g. LEDs or an infrared laser. Preferably, the light used for the exposure is a laser emitting near infrared light having a wavelength in the range from about 700 to about 1500 nm, e.g. a semiconductor laser diode, a Nd:YAG or a Nd:YLF laser. In accordance with the present invention, the energy density of the light used in the exposure step is 190 mJ/cm² or less, more preferably 180 mJ/cm² or less. Satisfactory results can also be obtained at an energy density of 160 mJ/cm² or less or even at 150 mJ/cm² or less.

Due to the heat generated during the exposure step, the hydrophobic thermoplastic polymer particles fuse or coagulate so as to form a hydrophobic phase which corresponds to the printing areas of the printing plate. Coagulation may result from heat-induced coalescence, softening or melting of the thermoplastic polymer particles. There is no specific upper limit to the coagulation temperature of the thermoplastic hydrophobic polymer particles, however the temperature should be sufficiently below the decomposition temperature of the polymer particles. Preferably the coagulation temperature is at least 10°C below the temperature at which the decomposition of the polymer particles occurs. The coagulation temperature is preferably higher than 50°C, more preferably above 100°C.

After exposure, the precursor is developed by means of a suitable processing liquid. In the development step, the non-exposed areas of the image-recording layer are removed without essentially removing the exposed areas, i.e. without affecting the exposed areas to an extent that renders the ink-acceptance of the exposed areas inacceptable. The processing liquid can be applied to the plate e.g. by rubbing in with an impregnated pad, by dipping, (spin-)coating, spraying, pouring-on, either by hand or in an automatic processing apparatus. The treatment with a processing liquid may be combined with mechanical rubbing, e.g. by a rotating brush. The developed plate precursor can, if required, be post-treated with rinse water, a suitable correcting agent or preservative as known in the art. During the development step, any water-soluble protective layer present is preferably also removed.

Suitable processing liquids are plain water or aqueous solutions, e.g. a gumming solution or an alkaline solution. Gumming solutions which are suitable as processing liquid preferably have a pH between 4 and 10 and have been described in EP-A 1 342 568. In a preferred embodiment, the processing step of the exposed plate is carried out using a gumming unit as shown in Figure 1. The gumming unit comprises (i) rollers 1 to 6 for transporting the plate through the device, (ii) spray tubes 7, 8 and 9 for applying the gum liquid and (iii) scrub rollers 10.

The embodiment using an alkaline solution is now described in more detail. A preferred aqueous alkaline solution has a pH of at least 10, more preferably at least 11, most preferably at least 12. In a preferred embodiment the pH is comprised between 10 and 14. Preferred aqueous alkaline solutions are buffer solutions such as for example silicate-based developers or developer solutions comprising phosphate buffers. Silicate-based developers which have a ratio of silicon dioxide to alkali metal oxide of at least 1 are advantageous because they ensure that the alumina layer (if present) of the substrate is not damaged. Preferred alkali metal oxides include Na₂O and K₂O, and mixtures thereof. A particularly preferred silicate-based developer solution is a developer solution comprising sodium or potassium metasilicate, i.e. a silicate where the ratio of silicon dioxide to alkali metal oxide is 1.

In addition to alkali metal silicates, the developer may optionally contain further components, such as buffer substances, complexing agents, antifoams, organic solvents in small amounts, corrosion inhibitors, dyes, surfactants and/or hydrotropic agents as known in the art.

The development is preferably carried out at temperatures of from 20 to 40°C in automated processing units as customary in the art. For regeneration, alkali metal silicate solutions having alkali metal contents of from 0.6 to 2.0 mol/l can suitably be used. These solutions may have the same silica/alkali metal oxide ratio as the developer (generally, however, it is lower) and likewise optionally contain further additives. The required amounts of regenerated material must be tailored to the developing apparatuses used, daily plate throughputs, image areas, etc. and are in general from 1 to 50 ml per square meter of plate precursor. The addition of replenisher can be regulated, for example, by measuring the conductivity of the developer as described in EP-A 0,556,690.

In accordance with the present invention, the developed plate is subjected to a mild post-baking step during a baking period of two minutes or less, i.e. between 5 seconds and 2 minutes. Preferably the baking period is less than one minute, more preferably less than 30 seconds. The developed plate can be dried before baking or is dried during the baking process itself. During the baking step, the plate is heated up to a baking temperature which is higher than the glass transition temperature of the thermoplastic particles. A preferred baking temperature is above 50°C, more preferably above 100°C. 'Baking temperature' as used herein refers to the temperature of the plate during the baking process. In a preferred embodiment, the baking temperature does not exceed 300°C during the baking period. More preferably, the baking temperature does not exceed 250°C, even not 220°C. Baking can be done in conventional hot air ovens or by irradiation with lamps emitting infrared light as disclosed in EP-A 1 506 854.

The baking temperature can be measured by means of one or more temperature probes, e.g. thermocouples, preferably fixed to the backside of the support. Since the coating is very thin (typically less than 1 µm) relative to the support, the temperature of the coating is essentially equal to the temperature of the support. Especially when using large plates, it may be observed that the temperature profile (temperature versus time) during the baking process at one spot on the plate, e.g. near the edge, is different from the temperature profile at another spot, e.g. near the center of the plate. In such case, it is preferred that the temperature at any spot on the plate, does not exceed a temperature of 300°C, more preferably a temperature of 250°C and most preferably a temperature of 200°C.

In a preferred embodiment, the exposure step, the processing step and the baking step are carried out in an integrated plate-making apparatus (Figure 2). The integrated plate-making apparatus comprises a plate-setter (**1**), a processing unit (**2**) and a small baking unit (**3**). The plate precursor which has been exposed in the plate-setter is mechanically conveyed via transferring means A to the processing unit which is further coupled via transferring means B to the baking unit. After developing the exposed plate in the processing unit, the developed plate is then mechanically conveyed via transferring means B to the baking unit. The short baking step according to the present invention allows the use of a small baking unit (the sizes of the different units of the plate-making apparatus are indicated on the figure in cm). The plate then travels through the baking unit and leaves said unit within a time period of two minutes or less. The baking unit may further comprise a cooling zone so that the plate temperature is reduced before the plate leaves the baking unit. Furthermore, the baking unit is preferably equipped with an exhaust which removes volatile compounds that may be released from the plate material. The exhaust preferably comprises an easily exchangeable filter.

The printing plate thus obtained can be used for conventional, so-called wet offset printing, in which ink and an aqueous dampening liquid are supplied to the plate. Another suitable printing method uses so-called single-fluid ink without a dampening liquid. Suitable single-fluid inks have been described in US 4,045,232; US 4,981,517 and US 6,140,392. In a most preferred embodiment, the single-fluid ink comprises an ink phase, also called the hydrophobic or oleophilic phase, and a polyol phase as described in WO 00/32705.

### EXAMPLES

### 1. Preparation of the lithographic support.

A 0.30 mm thick aluminum foil was degreased by immersing the foil in an aqueous solution containing 40 g/l of sodium hydroxide at 60°C for 8 seconds and rinsed with demineralized water for 2 seconds. The foil was then electrochemically grained during 15 seconds using an alternating current in an aqueous solution containing 12 g/l of hydrochloric acid and 38 g/l of aluminum sulfate (18-hydrate) at a temperature of 33°C and a current density of 130 A/dm². After rinsing with demineralized water for 2 seconds, the aluminum foil was then desmutted by etching with an aqueous solution containing 155 g/l of sulfuric acid at 70°C for 4 seconds and rinsed with demineralized water at 25°C for 2 seconds. The foil was subsequently subjected to anodic oxidation during 13 seconds in an aqueous solution containing 155 g/l of sulfuric acid at a temperature of 45°C and a current density of 22 A/dm², then washed with demineralized water for 2 seconds and post-treated for 10 seconds with a solution containing 4 g/l of polyvinylphosphonic acid at 40°C, rinsed with demineralized water at 20°C during 2 seconds and dried. The support thus obtained has a surface roughness Ra of 0.21 µm and an anodic weight of 4 g/m² of Al₂O₃.

### 2. Preparation of the printing plate precursor.

A printing plate precursor was produced by applying a coating onto the above described lithographic support. The aqueous coating solution had a pH of 3.55 and comprised the compounds listed in Table 1. After drying, the coating weight was 0.678 g/m².

**Table 1: composition of the dry coating.**

| INGREDIENTS | wt.% |
|---|---|
| Styrene/acrylonitrile copolymer (1) | 82.18 |
| Cu-phtalocyanine pigment (2) | 2.97 |
| Triethylammonium salt of IR-1 (3) | 7.92 |
| Polyacrylic acid binder (4) | 5.94 |
| Zonyl FSO 100 (5) | 1.00 |

| | |
|---|---|
| (1) weight ratio 60/40, stabilized with an anionic wetting agent; particle size of 50 nm, measured with a Brookhaven BI-90 analyzer, commercially available from Brookhaven Instrument Company, Holtsville, NY, USA. (2) Cab O Jet 250 from Cabot Corporation, added as 5% aqueous dispersion. (3) infrared dye defined above. (4) Aquatreat AR-7H from National Starch & Chemical Company, Mw = 500 000 g/mol. (5) Surfactant from Dupont | |

### 3. Preparation of the printing plates.

The obtained printing plate precursors were exposed with a CREO Trendsetter TE318 (40W) (plate-setter available from Creo, Burnaby, Canada), operating at an energy density of respectively 140 mJ/cm² (comparative printing plate 1 and invention printing plate 3) and 200 mJ/cm² (comparative printing plate 2) and at 150 rpm (Table 2).

After imaging, the printing plate precursors 1-3 were processed in an Agfa VA88 processor, operating at a speed of 1 m/min and at 22°C, and using Agfa TD1000 as developer solution and RC520 as gum solution; both trademarks of Agfa.

Printing plates 1 and 2 were mounted as such on the printing press while invention printing plate 3 was baked prior to mounting it on the press (Table 2). The baking step of invention printing plate 2 was carried out by heating the plate with an infrared radiation source at a temperature of 200°C and a dwell-time of the baking step of 20 seconds.

**Table 2: applied energy density and baking conditions.**

| Printing plate | Applied energy density mJ/cm² | Baking temperature °C | Baking periods |
|---|---|---|---|
| Comparative printing plate 1 (1) | 140 | - | - |
| Comparative printing plate 2 (1) | 200 | - | - |
| Invention Printing plate 3 | 140 | 200 | 20 |

| | | | |
|---|---|---|---|
| (1): the comparative printing plates 1 and 2 are not baked. | | | |

### 4. Print results.

The obtained printing plates were mounted on a Drent printing press (available from Drent Goebel), and a print job was started using Arets UV cyan EXC ink (trademark of Arets Graphics) and 2.5% FS405 in 10% isopropanol as a fountain liquid.

The lithographic properties of the plates were determined by visual examination of the prints after respectively 10.000 sheet and 55.000 sheet. The quality of the coating was determined by inspection of the rendering of a 10% screen of 200 lpi on print.

The results are presented in Table 3 and Figures 3 A and B: at an exposure density of 140 mJ/cm² and 200 mJ/cm² the rendering of a 10% screen of 200 lpi on print measured after 10.000 sheet is similar for the three plates (Figure 3A, 1=printing plate 1,. 2=printing plate 2 and 3=printing plate 3). Furthermore, the rendering of a 10% screen of 200 lpi on print measured after 55.000 sheet of invention printing plate 3 (Figure 3B,3), which has been underexposed and baked, is similar to comparative printing plate 2 (Figure 3B,2) which has been exposed at 200 mJ/cm² while the rendering of the 10% screen of 200 lpi on print after 55.000 sheet of comparative printing plate 1 (Figure 3B,3) which has been exposed at 140 mJ/cm² but was not baked, is damaged and almost not present any more on print. Thus, the mechanical and chemical resistance of the (underexposed) lithographic image exposed at an energy density of 140 mJ/cm² is unsufficient to retain an acceptable coating quality of the plate during printing while the mild post-baking step - whithout prejudice to the scope of our claims - seems to compensate for the underexposure.

**Table 3: rendering of a 10% screen of 2001pi on print.**

| | Rendering of a 10% screen of 2001pi on print(1) | |
|---|---|---|
| | After 10000 sheet | after 55000 sheet |
| Comparative printing plate 1 | + | - |
| Comparative printing plate 2 | + | + |
| Invention Printing plate 3 | + | + |

| | | |
|---|---|---|
| (1) +: indicates that the 10% screen of 200 lpi on print is unaffected. -: indicates that the 10% screen of 200 lpi on print is damaged. | | |

## Claims

1. A method for making a lithographic printing plate comprising the steps of :
i) providing a lithographic printing plate precursor comprising
- a support having a hydrophilic surface or which is provided with a hydrophilic layer, and
- a coating provided on said hydrophilic surface or said hydrophilic layer,
wherein the coating comprises an image recording layer comprising hydrophobic thermoplastic polymer particles and
wherein the image recording layer or an optional other layer of said coating further comprises an infrared light absorbing agent;
ii) image-wise exposing the precursor to infrared light having an energy density of 190 mJ/cm² or less;
iii) developing the exposed precursor by removing unexposed areas in a processing liquid;
iv) baking the plate thus obtained by keeping the plate at a temperature above the glass transition temperature of the thermoplastic particles during a period between 5 seconds and 2 minutes.

2. A method according to claim 1 wherein the energy density is 180 mJ/cm² or less.

3. A method according to claim 1 wherein the energy density is 160 mJ/cm² or less.

4. A method according to claim 1 wherein the energy density is 150 mJ/cm² or less.

5. A method according to any of the preceding claims wherein the baking period is less than 1 minute.

6. A method according to any of the preceding claims wherein the baking period is less than 30 seconds.

7. A method according to any of the preceding claims wherein the temperature of the plate does not exceed 300°C during the baking period.

8. A method according to any of the preceding claims wherein the temperature of the plate does not exceed 250°C during the baking period.

9. A method according to any of the preceding claims wherein the temperature of the plate does not exceed 220°C during the baking period.

10. A method according to any of the preceding claims wherein the hydrophobic thermoplastic polymer particles have an average particle size comprised between 40 nm and 70 nm.

11. A method according to any of the preceding claims wherein the image-recording layer further comprises a binder and wherein the amount of the hydrophobic thermoplastic polymer particles is at least 70 % by weight relative to the image-recording layer.

12. A method according to any of the preceding claims wherein the processing liquid is water or an aqueous solution.

13. A method according to any of the preceding claims wherein the processing liquid is a gum solution having a pH between 4 and 10.

14. A method according to any claims 1-12 wherein the processing liquid is an alkaline solution having a pH between 10 and 14.

15. A method according to any of the preceding claims wherein a plate-making apparatus is used, said plate-making apparatus comprising
a. a plate-setter for performing step ii),
b. a processing unit for performing step iii),
c. and a baking unit for performing step iv),
and wherein the plate is mechanically conveyed from the platesetter to the processing unit and from the processing unit to the baking unit.

16. A method of lithographic printing comprising the steps of
i) making a lithographic printing plate by a method according to any of the preceding claims;
ii) mounting the plate on a plate cylinder of a lithographic printing press;
iii) supplying ink and fountain solution to the plate;
iv) transferring the ink to paper.

## Patentansprüche

1. Ein die nachstehenden Schritte umfassendes Verfahren zur Herstellung einer lithografischen Druckplatte :
i) Bereitstellen einer lithografischen Druckplattenvorstufe, die
- einen Träger mit einer hydrophilen Oberfläche oder einen mit einer hydrophilen Schicht versehenen Träger und
- eine auf die hydrophile Oberfläche oder die hydrophile Schicht aufgebrachte Beschichtung umfasst,
wobei die Beschichtung eine hydrophobe thermoplastische Polymerteilchen enthaltende Bildaufzeichnungsschicht umfasst und die Bildaufzeichnungsschicht oder eine eventuelle andere Schicht der Beschichtung ferner einen IR-Absorber enthält,
ii) bildmäßige Belichtung der Vorstufe mit Infrarotlicht mit einer Energiedichte von höchstens 190 mJ/cm²,
iii) Entwicklung der belichteten Vorstufe durch Entfernung der unbelichteten Bereiche in einer Entwicklerflüssigkeit und
iv) Einbrennen der so erhaltenen Platte, indem die Platte bei einer oberhalb des Einfrierpunktes der thermoplastischen Teilchen liegenden Temperatur über einen Zeitraum von 5 Sekunden bis 2 Minuten gelagert wird.

2. Verfahren nach Anspruch 1, **dadurch gekennzeichnet, dass** die Energiedichte höchstens 180 mJ/cm² beträgt.

3. Verfahren nach Anspruch 1, **dadurch gekennzeichnet, dass** die Energiedichte höchstens 160 mJ/cm² beträgt.

4. Verfahren nach Anspruch 1, **dadurch gekennzeichnet, dass** die Energiedichte höchstens 150 mJ/cm² beträgt.

5. Verfahren nach einem der vorstehenden Ansprüche, **dadurch gekennzeichnet, dass** der Einbrennzeitraum weniger als 1 Minute beträgt.

6. Verfahren nach einem der vorstehenden Ansprüche, **dadurch gekennzeichnet, dass** der Einbrennzeitraum weniger als 30 Sekunden beträgt.

7. Verfahren nach einem der vorstehenden Ansprüche, **dadurch gekennzeichnet, dass** die Plattentemperatur während des Einbrennzeitraums nicht über 300°C hinauskommt.

8. Verfahren nach einem der vorstehenden Ansprüche, **dadurch gekennzeichnet, dass** die Plattentemperatur während des Einbrennzeitraums nicht über 250°C hinauskommt.

9. Verfahren nach einem der vorstehenden Ansprüche, **dadurch gekennzeichnet, dass** die Plattentemperatur während des Einbrennzeitraums nicht über 220°C hinauskommt.

10. Verfahren nach einem der vorstehenden Ansprüche, **dadurch gekennzeichnet, dass** die mittlere Teilchengröße der hydrophoben thermoplastischen Polymerteilchen zwischen 40 nm und 70 nm liegt.

11. Verfahren nach einem der vorstehenden Ansprüche, **dadurch gekennzeichnet, dass** die Bildaufzeichnungsschicht ferner ein Bindemittel enthält und die Menge der hydrophoben thermoplastischen Polymerteilchen zumindest 70 Gew.-%, bezogen auf die Bildaufzeichnungsschicht, beträgt.

12. Verfahren nach einem der vorstehenden Ansprüche, **dadurch gekennzeichnet, dass** die Entwicklerflüssigkeit Wasser oder eine wässrige Lösung ist.

13. Verfahren nach einem der vorstehenden Ansprüche, **dadurch gekennzeichnet, dass** die Entwicklerflüssigkeit eine Gummierlösung mit einem pH zwischen 4 und 10 ist.

14. Verfahren nach einem der Ansprüche 1 bis 12, **dadurch gekennzeichnet, dass** die Entwicklerflüssigkeit eine alkalische Lösung mit einem pH zwischen 10 und 14 ist.

15. Verfahren nach einem der vorstehenden Ansprüche, **dadurch gekennzeichnet, dass** ein Plattenherstellungsgerät verwendet wird, wobei das Plattenherstellungsgerät folgende Elemente umfasst :
a. einen Plattenbelichter zum Ausführen von Schritt ii),
b. eine Entwicklungseinheit zum Ausführen von Schritt iii) und
c. eine Einbrenneinheit zum Ausführen von Schritt iv),
und wobei die Platte mechanisch vom Plattenbelichter zur Entwicklungseinheit und von der Entwicklungseinheit zur Einbrenneinheit gefördert wird.

16. Ein die nachstehenden Schritte umfassendes lithografisches Druckverfahren :
i) Herstellung einer lithografischen Druckplatte gemäß einem Verfahren nach einem der vorstehenden Ansprüche,
ii) Aufspannen der Platte auf einen Plattenzylinder einer lithografischen Druckpresse,
iii) Einfärben der Platte mit Druckfarbe und Benetzen der Platte mit Feuchtwasser und
iv) Übertragung der Druckfarbe auf Papier.

## Revendications

1. Un procédé pour la confection d'une plaque d'impression lithographique, comprenant les étapes ci-après :
i) la mise à disposition d'un précurseur de plaque d'impression lithographique, comprenant
- un support ayant une surface hydrophile ou un support revêtu d'une couche hydrophile et
- un revêtement appliqué sur la surface hydrophile ou la couche hydrophile,
**caractérisé en ce que** ledit revêtement comprend une couche d'enregistrement d'image contenant des particules d'un polymère hydrophobe thermoplastique et que la couche d'enregistrement d'image ou une éventuelle autre couche du revêtement contient en outre un agent absorbant la lumière infrarouge,
ii) l'exposition sous forme d'image du précurseur à de la lumière infrarouge présentant une densité énergétique maximale de 190 mJ/cm²,
iii) le développement du précurseur exposé par élimination des zones non exposées dans un liquide révélateur et
iv) la cuisson de la plaque ainsi obtenue en conservant la plaque à une température supérieure au point de transition vitreuse des particules thermoplastiques pendant 5 secondes à 2 minutes.

2. Procédé selon la revendication 1, **caractérisé en ce que** la densité énergétique maximale s'élève à 180 mJ/cm².

3. Procédé selon la revendication 1, **caractérisé en ce que** la densité énergétique maximale s'élève à 160 mJ/cm².

4. Procédé selon la revendication 1, **caractérisé en ce que** la densité énergétique maximale s'élève à 150 mJ/cm².

5. Procédé selon l'une quelconque des revendications précédentes, **caractérisé en ce que** le temps de cuisson est inférieur à 1 minute.

6. Procédé selon l'une quelconque des revendications précédentes, **caractérisé en ce que** le temps de cuisson est inférieur à 30 secondes.

7. Procédé selon l'une quelconque des revendications précédentes, **caractérisé en ce que** la température de la plaque pendant le temps de cuisson ne dépasse pas 300°C.

8. Procédé selon l'une quelconque des revendications précédentes, **caractérisé en ce que** la température de la plaque pendant le temps de cuisson ne dépasse pas 250°C.

9. Procédé selon l'une quelconque des revendications précédentes, **caractérisé en ce que** la température de la plaque pendant le temps de cuisson ne dépasse pas 220°C.

10. Procédé selon l'une quelconque des revendications précédentes, **caractérisé en ce que** la grandeur de particule moyenne des particules d'un polymère hydrophobe thermoplastique est comprise entre 40 nm et 70 nm.

11. Procédé selon l'une quelconque des revendications précédentes, **caractérisé en ce que** la couche d'enregistrement d'image contient en outre un liant et que la quantité des particules d'un polymère hydrophobe thermoplastique s'élève à au moins 70% en poids par rapport à la couche d'enregistrement d'image.

12. Procédé selon l'une quelconque des revendications précédentes, **caractérisé en ce que** le liquide révélateur est de l'eau ou une solution aqueuse.

13. Procédé selon l'une quelconque des revendications précédentes, **caractérisé en ce que** le liquide révélateur est une solution de gommage ayant un pH compris entre 4 et 10.

14. Procédé selon l'une quelconque des revendications 1 à 12, **caractérisé en ce que** le liquide révélateur est une solution alcaline ayant un pH compris entre 10 et 14.

15. Procédé selon l'une quelconque des revendications précédentes, **caractérisé en ce qu'**il est utilisé un appareil de confection de plaques comprenant les éléments suivants :
a. une unité d'exposition directe de plaques destinée à l'exécution de l'étape ii),
b. une développeuse destinée à l'exécution de l'étape iii) et
c. une unité de cuisson destinée à l'exécution de l'étape iv),
et que la plaque est transportée de façon mécanique de l'unité d'exposition vers la développeuse et de la développeuse vers l'unité de cuisson.

16. Un procédé d'impression lithographique, comprenant les étapes ci-après :
i) la confection d'une plaque d'impression lithographique selon un procédé selon l'une quelconque des revendications précédentes,
ii) le calage de la plaque sur un cylindre porte-plaque d'une machine à imprimer lithographique,
iii) l'encrage de la plaque et le mouillage de la plaque et
iv) le transfert de l'encre sur du papier.
